

## UNITED STATES PATENT OFFICE

2,344,260

## ALKALI SALTS OF FATTY AMINO COMPOUNDS

Willard L. Morgan, Edgewood, and Earle Davis McLeod, Rumford, R. I., assignors to Arnold, Hoffman & Co. Incorporated, a corporation of Rhode Island

No Drawing. Application April 14, 1941,  
Serial No. 388,559

14 Claims. (CL. 260—404.5)

This invention relates to salts of condensation products which are suitable as assistants for the modification of the properties of textile fibers, which assistants cannot be removed by washing or dry cleaning and which have no deleterious effects on the fastness to light of colored fabrics. Many materials have been used as textile assistants for altering the softness, the easy wetting or the repellency of textile fibers, but each has been subject to some fault, thus tallow, oils or sulfonated tallow have long been used in the finishing of textiles for softening effects, but these effects are not permanent and are lost the first time the goods are washed. These materials also suffer from rancidity or objectionable odor development in the goods. Fatty alcohols and simple aliphatic amides, which do not become rancid, have also been used as textile softeners, but these also wash out.

It is known that the quaternary salts of aliphatic amides which are formed by the reaction of aliphatic amides with acids as well as similar fatty quaternaries produced from pyridines or the betaines and aliphatic imidazoles solubilized as salts by treatment with acids are useful as textile modifying agents, and in particular as textile softeners, particularly as these materials alter or soften the fibers and cannot thereafter be washed off. In a similar way quaternary salts have been formed from these various aliphatic amino bases by reaction of solubilizing acids, such as, acetic, hydrochloric, etc., and also by treatment with alkylating agents such as diethyl sulfate, ethyl chloride or chloroacetic acid. The quaternary salts of fatty acid condensations with aliphatic polyamines have particularly been used for these purposes.

As a consequence of the marked advantages secured with the aliphatic amino quaternaries on textiles, their use has been very extensive, but it has been found, unfortunately, when used on printed or colored cloth that all of these aliphatic amino compounds have caused a very serious alteration in the light fastness of the colored textiles. In the case of commercial colors or direct dyestuffs and the basic type dyestuffs these effects have been particularly severe and in many cases the resistance to fading is reduced to practically nil. Direct dyestuffs are perhaps used more than any other dyestuffs in the cotton trades because of their general brightness and generally good resistance to light fading. The serious reduction in light fastness arising with the various types of aliphatic amino quaternary substances is also found with acid type dyestuffs

which are the main type used on wool fabrics. Other types of dyestuffs, such as rapidogens, indigosols and vats, as well as acetate colors are affected in many cases although not universally as it appears to be particularly true in the direct, basic and acid colors. While there is some slight variation in the deleterious effects of the various types of aliphatic amino quaternary substances on dyestuffs, none of these is in any way completely free of the difficulty and the use of any of them on colored goods constitutes a considerable trade hazard and has been the source of loss in the textile trade and unsatisfaction to the consumer employing the goods because of a very poor light resistance. As an example, a fabric dyed with Diphenyl Blue Green BL, direct dyestuff, E. I. du Pont de Nemours, which readily gives a 40-hour fading test in an ultraviolet fadeometer or resists a three months' outdoor service without any evidence of fading will after treatment in a 1/4% solution or less of any of the aliphatic amino quaternaries described show evidence of failure within a five hour fading test, and at forty hours the dyestuff is almost completely faded out.

It is an object of this invention to provide a new class of textile assistants, such as wetting, washing, softening, lubricating and waterproofing agents.

It is also an object of this invention to provide a new class of textile assistants, such as wetting, washing, softening, lubricating, and waterproofing agents having improved properties and characterized by not having any deleterious fading effect on colored textile materials.

As a further object of our invention, we describe new salts of aliphatic amino compounds useful as textile assistants which may be easily applied from aqueous solutions to give finishes on cloth of a maximum softness and which effects are completely resistant to washing and to dry cleaning, and at the same time free of any deleterious effects upon the fading resistance of the dyestuffs employed on the colored cloth.

A still further object of our invention is to describe new salts of aliphatic amino compounds which may be used to lubricate either yarns or fabrics so as to make the mechanical flow of these in weaving or sewing proceed smoothly.

We have found that the deleterious effects on fading of dyestuffs by the ordinary aliphatic amino quaternary acid salts which have generally been described as cationic active materials are due to their reaction with the dyestuff and the formation of new dyestuffs of completely altered

and practically invariably decreased fading resistance to light. New dyestuffs are formed by reaction of the quaternary nitrogen acid salts with dyestuffs carrying sulphonic acid groups, which is particularly true for most all direct dyestuffs and acid type dyestuffs. In these dyestuffs the large color group carrying the sulphonic acid group forms a negative ion in water solution, and this negative ion reacts with the large positive substituted ammonium quaternary ion or cation formed from the quaternary compounds when they are dissolved in water. The cation carries practically all of the organic compound attached to the pentavalent nitrogen, the entire group carrying a positive charge and only the acid radical coming from the solubilizing acid goes into the negative ion formed, thus we may typify the reaction of the dyestuff with a quaternary aliphatic amino acid salt by the following reactions, where  $D$  is the large organic dyestuff complex carrying the sulphonic acid group. The pentavalent nitrogen or quaternary compound is indicated as carrying three substituent organic radicals ( $R$ ) and a hydrogen which latter arises from the solubilizing acid. The other radical, indicated by  $A$ , hooked to the pentavalent nitrogen arises from the solubilizing acid which, for instance, may be acetic acid in which case  $A$  is an acetate radical.



That the last reaction does occur can readily be seen when solutions of direct dyestuffs and of cation active materials are mixed as there is an immediate coprecipitation resulting in the formation of a new dyestuff which is oil soluble. Oil soluble dyes in general have always been noted for very poor light fastness.

The textile modifying agents proposed by this invention are new alkali salts of aliphatic amino compounds containing hydroxylated, carboxylated, or amino side chains characterized by the fact that the aliphatic amino acid group forms in water a large negative ion. In these compounds nitrogen is only found in a trivalent condition and there are no pentavalent or quaternary nitrogens present. The new compounds which we propose to use as textile modifying agents and softening agents are further characterized by the presence of one or more groups of the following types:



As will be seen these are amide and amidine groups, in which the acid hydrogen attached to the nitrogen has been replaced by an alkali base indicated by ME, such as sodium or potassium. We have found that in aliphatic amide and aliphatic amidine compounds which carry the respective groups.



that the hydrogen is a weak acidic hydrogen which can readily be replaced by the alkalies

when these compounds are treated with strong alkalis.

We may make our new alkali salts of aliphatic amides and amidines by reacting a wide range of aliphatic amide and amidine types of substances with strong alkalis. In general, the new softeners which we described are of the following general formula:



Y is used to represent either oxygen ( $=O$ ) or an imide group ( $=NH$ ) and t is a small whole integer being either 1 or 2. In the wide majority of our compounds  $R_1$  corresponds preferably to a saturated aliphatic chain containing 6 or more carbons, or it may also represent other hydrocarbon radicals of 6 or more carbons, such as cyclo alkyls, an unsaturated hydrocarbon, an aryl radical, or a residue from a terpene acid, and it may carry other substituted groups such as hydroxyl, carboxyl, or chlorine. In each case the corresponding acid and acid chloride esters or nitriles may be used as a source to introduce this radical into our condensation products as will be shown later.

The alkali salts of the aliphatic amides are made by treating aliphatic amide products with strong alkalies. We may make our aliphatic amides, where  $t$  is equal to 1, by condensing suitable acids with the alkylolamines, amino acids, and polyamines. As suitable acids for condensing to these products, we prefer those containing 6 or more carbons and preferably saturated aliphatic acids, such as lauric, stearic, and palm oil acids, although we may use the unsaturated or substituted fatty acids such as ricinoleic, oleic, sebacic, or chlorostearic; or the cyclo aliphatic, aromatic, or resin acids may also be used, such as naphthenic, benzoic, creositic, and abietic, or the resin acid secured from rosin and maleic anhydride.

The alkali salts of the aliphatic amidine compounds are made by reacting strong alkali solutions on the condensates secured from aliphatic nitriles with amines, alkylolamines, amino acids or polyamines.

The group  $X$  is of the nature depending entirely upon the type of amine used in the initial condensations with the fatty compounds, and  $X$  must carry hydroxyl, carboxyl, or amino groups. Thus the organic acids may be condensed with monoethanolamine in which case  $X$  is an ethanol group, and similar type compounds may be secured using other primary amino alkylol compounds, such as, 2 amino, 2 ethyl, 1,3 propanediol; 2 amino, 2 methyl, 1,3 propanediol; 2 amino 1 pentanol; 3 amino, 2 butanol; 2 amino, 2 methyl, 1 propanol; and trimethanol amino methane.  $X$  may be a methylol group where aliphatic amides are reacted with formaldehyde. In all these cases our alkali salts are made by treating the condensates with strong alkalies. Where  $X$  carries a carboxyl group one convenient method of securing this is by condensing an amino acid with the other organic acid, and as suitable amino acids we may use amino acetic acid or glutamic acid. Our alkali salts can readily be prepared

also from compounds in which X carries free  
70 amino groups, such as may be secured by con-  
densing the organic acids with any of the aliphatic polyamines or substituted polyamines,  
such as diethylene triamine; triethylene tetra-  
75 ramine; tetraethylene pentamine; hexaethylene diamine; hydroxy ethyl ethylene diamine; ethyl

ethylene diamine; 2,2 dimethyl, 1,3 diamino propane; 1,3 diamino isopropanol; beta,beta diamino diethyl ether; and beta,beta, diamino diethyl thioether. In general we have found that where we react aliphatic amines with fatty acids that the alkali salts of the resulting aliphatic amide are not water soluble.

The new alkali salts of aliphatic amide and aliphatic amidine compounds may carry more than one of the characteristic respective groups:



Such compounds, in which  $t$  is equal to 2, can readily be made by reacting polyamines with more than one mol of organic acids. We may secure a similar condensate where  $t$  is equal to 2 by further condensing a polyamine organic acid condensate with formaldehyde.

The aliphatic amide and amidine condensations are readily carried out by heating the organic acids and amines at temperatures from 130 to 200° C. until the reaction is complete as shown by the loss of water. The molten materials are then cooled down to below 100° C. and while still molten are mixed with strong alkali solutions of caustic soda or potassium hydroxide. Further water is then immediately stirred in in order to secure soaplike pastes which can thereafter be diluted with further water at the time these materials are to be applied to the textiles.

The formation of the alkali salts makes the basic organic compound soluble in water. The alkali salts of these compounds are found to show high substantivity to various textile fibers, such as cotton, viscose, cellulose acetate, rayon, jute, etc., and to give textile treatments which are permanent to washing and dry cleaning. In general, while the larger molecules are desirable for substantivity, they are also inclined to be water insoluble, but by the formation of our alkali salts by treating the original condensations with strong alkalis, we are able to increase their solubility in water. In general we find the solubility in water to also improve as the number of amino, carboxyl, and hydroxyl groups are increased and as the molecular weight of the fatty acid, etc., is decreased.

The aliphatic amide and amidine groups,



present in the original aliphatic condensates are weak acids and in general the weak acidic hydrogen reacts readily only with the strong alkalies, such as, sodium and potassium hydroxide. However, where the organic acid group present is not too large, or for instance, contains 12 carbons or less, such as in the lauric compounds, the water solubility of the initial organic condensates is considerable, and in these cases we may form alkali salts between these bases and weaker alkalies, such as ammonia or the various alkylol amines and alkyl polyamides such, for instance, as monoethanolamine or diethylene triamine. In general, then we may replace the sodium or potassium hydroxide by these materials and form the corresponding am-

monium and amine salts, but in general we prefer to use the stronger sodium and potassium hydroxide. As the aliphatic amino compounds are all very weak acids, the alkali salts of these compounds all show an alkaline reaction in water solution. In some cases our alkali salts of the aliphatic amino compounds can be made by mixing with strong alkaline salts which provide free alkalies when dissolved in water. Examples of this type are soaps and the sodium salts of sulphonated alkylated biphenyl compounds.

It is apparent by reason of the large molecular weight of our aliphatic amino compounds that the actual amount of alkali needed to convert these into the alkali salts is a relatively small amount as will be apparent in the examples detailed hereafter. Our new alkali salts of aliphatic amino compounds possess marked emulsifying properties, and it is possible to readily emulsify oils or waxes in pastes of these materials. These give very stable emulsions when diluted with water. In fact, we find that our alkali salts will frequently emulsify considerable quantities of the aliphatic amino compound bases which have not been converted into the alkali salts, thus, making it possible to use less than molal quantities for the securing of apparently water soluble or at least stable emulsions of these products. Many water soluble compounds, such as, hydroscopic agents, for example, diethylene glycol, dextrose, or urea can, of course, be added directly to the water pastes of our new alkali salts where it is desirable to use these on textiles in conjunction with the new textile modifying agents.

As can be seen from the nature of our general formula, there are not present in any of our new substantive treating agents any pentavalent or quaternary nitrogens and it is apparent that our new alkali salts, when dissolved in water, ionize in a completely different way from the quaternary or cation active materials in that our products ionize into a positive alkali cation and a large organic ion which is charged with a negative charge. Since the dyestuff ionizes in a similar way, there is no tendency for negative ions of our textile treating agents to combine with the negative ion of the dyestuff, and the nature of the original dyestuff is completely preserved; thus, it is found that when our new softeners and other textile modifying agents are put onto dyed cloth irrespective whether the dyestuff used on the cloth is direct dyestuff, acid, vat, indigosol, rapidogen, or other types of dyestuff, the resistance to fading on exposure to light is found to be the same as that exhibited by the untreated colored cloth.

In addition to many of our materials having a marked permanent softening effect on the textiles, we may apply many of these as lubricating agents to yarns or textile constructions, or we may apply them to increase the rewetting or absorbability of the cloth or conversely in some cases we may apply them as waterproofing effects, all of which will be apparent in the examples hereafter described. Many of our compounds are also useful as detergents inasmuch as many of the products show distinct soaplike characteristics in their physical natures and operate very satisfactorily as cleaning agents for the washing of textiles and other materials.

The invention will be further illustrated but is not limited by the following examples in which the quantities are stated in parts by weight:

**Example 1**

31.7 parts (1 mol) of an aliphatic acid amide condensate of formula:



was made by condensing equimolar quantities of stearic acid and monoethanolamine at temperatures between 130° C. and 200° C. To this condensate, at temperatures below 100° C., were added 3.5 parts (1 mol) of 100% ammonium hydroxide as a 28% ammonia solution and the mix well stirred. Water was further added to this base to form a creamy paste of approximately 30% solids. This stock paste may then be further diluted at the time of use to give solutions containing  $\frac{1}{2}$  to 1% solids, and such solutions may be used to treat textile fibers whereupon, after drying, the fabrics will be found to be softened and somewhat water resistant. The softener is wash resistant and will not affect the light fastness of any dye which may be used on the cloth.

The water soluble ammonium salt of the aliphatic amino compound produced and used as a softener in this example is of the following formula:

**Example 2**

An aliphatic acid amide of formula:



was made by condensing equimolar quantities of lauric acid and monoethanolamine between temperatures of 130° C. and 200° C. To 24.3 parts (1 mol) of the above condensate, melted and at a temperature below 100° C., were added 5.6 parts (1 mol) of solid potassium hydroxide as a 45% solution and the paste formed thoroughly stirred. The alkali salt formed was further diluted with hot water to give a white paste of approximately 25% solids. This stock paste may then be further diluted at the time of use to give solutions containing  $\frac{1}{2}$  to 1% solids and such solutions may be used as softeners on textile yarns whereupon, after drying, the yarns will be found to be softened, that the softener wash resistant, and that this softener will have no effect on the light fastness of any dyes which may subsequently be used. Application of 1 to 10% of the alkali salt by weight to the weight of the yarn supplies a very satisfactory lubricating effect which facilitates the use of these yarns either in knitting or spinning operations. The aqueous solutions of the above compound show this material to be a good wetting agent for use on greige goods and other fabrics. In solutions of  $\frac{1}{2}$  to 1% it shows equally as good washing properties on wool or cotton as is shown by ordinary soaps.

The water soluble potassium salt of the aliphatic amino compound produced above is of the following formula:

**Example 3**

An aliphatic amino compound was made by condensing equimolar proportions of lauric acid

and 2 amino, 2 methyl, 1,3 propanediol at temperatures between 130° C. and 200° C. during which time the amide is formed. To 28.7 parts (1 mol) of the above melted compound and be-

5 low 100° C. were added 5.6 parts (1 mol) of solid potassium hydroxide as a 45% solution. This heavy base was thoroughly mixed and further diluted with water to form a 30% solid paste. This stock paste may further be diluted with water 10 at the time of use to give solutions containing  $\frac{1}{2}$  to 1% solids which will impart a soft hand to yarns or fabrics. The softness thus obtained will be wash resistant, show no odor development on aging, and in addition will not affect the light 15 fastness of any dyestuff used.

The potassium salt of the above aliphatic amino compound used as a softener in the above example is of the following formula:

**Example 4**

As another example of our alkali salts of aliphatic ethanol amides, we first prepare an aliphatic amide by condensing equimolar quantities of stearic acid and diethanolamine between temperatures of 130° C. to 200° C. followed by the addition of 1 mol or more of diethanolamine continuing heating between 130° C. to 200° C. during which time the excess diethanolamine reacts with the ethanol amide first formed and water is split out. To 45.6 parts (1 mol) of this ethanol condensate is added 4.0 parts (1 mol) of solid potassium hydroxide as a 50% solution. This heavy paste is thoroughly stirred and hot water added to give a 25% solids white paste. This stock paste 30 may be further diluted, when desired, with water to give solutions containing  $\frac{1}{2}$  to 1% solids. Solutions of these strengths, when used to soften yarns aid in further manipulations of yarns in weaving and sewing. The softening and lubricating effect produced on the yarns is wash resistant and when subsequently dyed will not affect the light fastness of the dye used.

**Example 5**

50 An aliphatic amino condensate was made by floating equimolar proportions of rosin acid and tetraethylene pentamine at temperatures between 130° C. and 200° C. The compound obtained was soft, semi-liquid in nature and dark 55 amber. The rosin condensate obtained above may be solubilized with potassium oleate soap, as for example, 1 part by weight of the rosin compound may be added to 4 parts of a 50% potassium oleate soap paste and the mixture thoroughly stirred at 60 a temperature of 60° C. to 80° C. during which time the rosin condensate will solubilize from the alkali obtained by the soap hydrolyzing in aqueous solutions. This paste may be further diluted to give a white stock paste of approximately 30% 65 solids. In use, this stock paste may be further diluted with water to give solutions containing 1 to 1½% solids. These solutions possess detergent properties as well as softening qualities and may be used in the washing and scouring of yarns 70 or fibers thereby leaving the yarns in a softened, cleaned condition for finishing. The softness imparted is resistant to washing and when further dyed will yield deeper shades with no effect on the light fastness of the dye that is used.

The salt of the rosin amine condensate formed

by the alkali obtained from the potassium oleate soap is of the following formula:



*Example 6*

An aliphatic amino condensate was prepared by condensing equimolar proportions of ricinoleic acid and diethylene triamine at temperatures between 130° C. and 200° C., during which time the amide was formed and 1 mol of water split out. The compound obtained was liquid at room temperatures. 3 parts by weight of the ricinoleic condensate obtained, which is liquid at room temperatures, were added to 1 part of a sodium salt of a sulphonated, alkylated, biphenyl compound, such as, the sodium salt of dibutyl-ortho-hydroxybiphenyl-disulfonic acid, dissolved as a 50% aqueous solution. The mixture was thoroughly stirred during which time the ricinoleic condensate was solubilized by the alkali salt used. The base was further diluted with water to give a stock paste of approximately 35% solids. In use, this paste may be further diluted to solutions containing 1/2 to 1% solids which solution possesses good wetting properties. Fabrics softened with these solutions re-wet easily, and by reason of this re-wettability the compound is applicable to "Sanforizing" operations. In addition, any dyestuff which may be used on the fabric is not affected in its light fastness by the softener used.

*Example 7*

370 parts (1 mol) of an aliphatic amino compound were made by condensing equimolar portions of stearic acid and diethylene triamine at temperatures between 130° C. and 200° C. The amide formed was light yellow with a melting point of 81° C. and possessed the following formula:



To 37.7 parts (1 mol) of the above condensate were added 4.0 parts (1 mol) of solid sodium hydroxide as a 50% solution. This base was thoroughly stirred and hot water added to give a 30% stock paste. This paste may be further diluted in use, and in strengths of 1/2 to 1% solids may be used for softening fabrics. Fabrics thus softened with these solutions will possess very good drape and be resistant to washing. No effect will be found on the light fastness of any dyes which may have been used on the fabric.

The sodium salt of the above aliphatic amino condensate is of the following formula:



*Example 8*

As a further example of our alkali salts of aliphatic amino compounds, we may first prepare a condensate of stearic acid and hydroxy ethyl ethylene diamine by heating equimolar proportions of the compounds between 130° C. and 200° C. during which time the amide is formed and one mol of water is split out. This condensate may be solubilized in water by the addition of strong alkalies as, for example, 37.8 parts (1 mol) may be solubilized by adding to the molten base at temperatures below 100° C. 5.6 parts (1 mol) of solid potassium hydroxide as a 45% solution. 75

This base may be further diluted with hot water to give a white paste of approximately 25% solids. The sodium salt of the above condensate possesses emulsifying properties and, as such, may be used to emulsify waxes, oils, or the non-soluble condensate described above. For example, as much as 4 parts by weight of the aliphatic amino condensate obtained above may be melted and added to 1 part of the anhydrous potassium salt in the form of a 30% paste and the mixture thoroughly stirred at temperatures between 60° C. and 80° C. During this time the 4 parts of base will be emulsified by the alkali salt and the mixture may then be further diluted with water to any desired concentration.

In use, the stock paste obtained may be further diluted with water to solutions containing 1/2 to 1% solids and thus used to impart softness to yarns or fabrics. Fabrics softened with this material possess a high degree of softness which is resistant to washing, and no effect on the light fastness of the dyestuff is obtained.

The alkali salt of the condensate obtained above, used as an emulsifier in this example, possesses the following formula:



*Example 9*

An aliphatic amino condensate was prepared by condensing 2 mols of stearic acid with one mol of 1,3 diamino isopropanol at temperatures between 130° C. and 200° C. during which time the distearyl amide condensate was obtained and 2 mols of water split out. The condensate was hard, light amber, and melted at 80° C. to 85° C. To 64.1 parts (1 mol) of the molten condensate at temperatures between 80° C. to 100° C. were added 11.2 parts (2 mols) of solid potassium hydroxide as a 45% solution. The mix was thoroughly stirred and further diluted with hot water to yield a 25% light amber paste. This stock paste may be further diluted by the addition of hot water to solutions containing 1/8 to 1/2 of 1% solids at the time of use. When used in these strengths, this compound will impart a marked softness to various fabrics, such as cotton, viscose, cellulose acetate, linen, jute, etc., and the softness thus obtained will be wash resistant and will have no effect on any dyes used on the fabric.

The potassium salt of the above condensate used in this example is of the following formula:



*Example 10*

A still further example of our alkali salts of amino compounds may be prepared by first condensing equimolar proportions of stearic acid and hydroxy ethyl ethylene diamine at temperatures between 130° C. and 200° C. The condensate obtained by this reaction is of the following formula:



This condensate may be further condensed with formaldehyde as, for example, 37.8 parts (1 mol) of the above condensate may be reacted with 15 parts (1/2 mol) of formaldehyde as a 40% solution at temperatures above 100° C. during which time

water is split out between secondary amino radicals and a compound of the following formula is formed:



This water insoluble condensate may be solubilized by the addition of strong alkali, as, for example, 76.8 parts (1 mol) of the melted compound at temperatures between 80° C. and 100° C. were thoroughly stirred with 4.0 parts (1 mol) of solid sodium hydroxide as a 50% solution. This alkali salt possessing the formula:



may be further diluted with hot water to give a white, creamy paste containing approximately 35% solids. The above sodium salt, when used in a dyebeck, in the ratio of 6 pounds of this paste to 1200 gallons (200ths of 1%) imparts a soft hand to fabrics which is resistant to washing and aging and has no effect on the resistance of fading of any dyestuff which might be used.

*Example 11*

In preparing aliphatic amino condensates we may also condense an amino acid with a fatty acid as, for example, by condensing equimolar proportions of lauric acid and alpha amino isocaproic acid (leucine) at temperatures between 130° C. and 200° C. during which time 1 mol of water is split out and a compound of the following formula is obtained:



This condensate may be solubilized with ammonium hydroxide by adding 3.5 parts (1 mol) of ammonium hydroxide as a 28% solution of ammonia to 31.3 parts (1 mol) of the condensate, molten and below 100° C. More than one mol of ammonium hydroxide is preferred to obtain good water solubility and the yellow paste obtained may be further diluted to approximately 35% solids. The stock paste thus made may be further diluted to concentrations of 1 to 1½% solids which solutions possess good wetting, foaming and detergent properties.

*Example 12*

An aliphatic amidine condensate may be prepared by heating equimolar proportions of lauric nitrile and diethylene triamine, during which time the diethylene triamine and lauric nitrile form a compound of the following formula:



This compound may be solubilized by treatment with strong alkali as, for example, 28.3 parts (1 mol) of the amidine condensate may be thoroughly mixed with 5.6 parts (1 mol) of solid potassium hydroxide as a 45% solution. The soluble alkali base obtained may be further diluted with water to concentration of 40% solids. This stock paste, in use, may be further diluted with water to solutions containing ½ to 1% solids

and as such used to impart softness to yarns or fabrics. The softness thus imparted is wash resistant, and the compound on the yarns or fabrics will have no effect on the light fastness of any dye which may be used.

The alkali salts of the aliphatic amidine obtained above has the following formula:



*Example 13*

As a further example of our alkali salts of poly amino condensates, we may first prepare the condensate of lauric acid and ethylene diamine by heating equimolar proportions at temperatures of 130° C. to 200° C. The condensate thus obtained is light yellow, melting at 124° C., and because of its high melting point is difficultly soluble. This condensate may be solubilized by treatment with strong alkali as, for example, 24.2 parts (1 mol) of the lauric condensate may be treated with 4.0 parts (1 mol) of solid sodium hydroxide as a 50% solution. This base, when thoroughly stirred, may be further diluted with hot water and on continual stirring will yield a smooth paste of approximately 30% solids. To 3 parts of this 30% solids paste is added one part by weight of diethylene glycol and the mixture is thoroughly stirred at temperatures between 60° C. and 80° C. This paste when used in the ratio of 2 to 6 pounds per 50 gallons of water imparts to hard, twisted, acetate fabrics a soft handle which is resistant to washing and gives a highly desirable drape. In addition there is no effect on the light fastness of any dyestuff which might be used. Used in the ratio of 4 to 6 pounds per 50 gallons this compound possesses wetting properties in aqueous solutions.

The alkali compound of the lauric condensate described above is of the following formula:



As many apparently widely different embodiments of this invention may be made without departing from the spirit and scope thereof, it is understood that we do not limit ourselves to the specific embodiments thereof except as defined in the appended claims.

We claim:

55. 1. A substituted amino compound of the following general formula:



60. in which Me represents an alkali metal, t is a small whole integer being 1 or 2, and in which R<sub>1</sub> represents a hydrocarbon radical of at least six carbon atoms and in which X is an alkyl group carrying a group selected from the groups consisting of hydroxyl, carboxyl, and amino groups.

65. 2. An organic amide of the following general formula:



70. in which Me represents an alkali metal and R<sub>1</sub> an organic acid residue of more than 6 carbons.

3. A stearo ethanol amide having the following formula:



in which Me is an alkali metal.

4. An organic amide of the following general formula:



in which Me represents an alkali metal and  $\text{R}_1$  an organic acid residue of more than 6 carbons.

5. A polyamino amide having the following formula:



in which Me is an alkali metal.

6. An organic amide of the following general formula:



in which Me represents an alkali metal and  $\text{R}_1$  an organic acid residue of more than 6 carbons.

7. A polyamino amide having the following formula:



in which Me is an alkali metal.

8. A substituted amino compound of the following general formula:



in which Me represents an alkali metal,  $t$  is a small whole integer being 1 or 2, and in which  $\text{R}_1$  represents a hydrocarbon radical of at least six carbon atoms and in which  $\text{X}$  is an alkyl group carrying a group selected from the groups consisting of hydroxyl, carboxyl, and amino groups.

10 9. Aliphatic alkylol amides in which the acid hydrogen attached to the amide nitrogen is replaced by an alkali metal.

15 10. The process of forming an alkylol amide compound in which alkylol amides of an organic acid of over six carbon atoms are reacted with an alkali metal hydroxide solution at a temperature below 100° C.

20 11. The process for forming an ethanol amide compound in which an organic acid of over six carbon atoms is reacted with monoethanolamine at 130° C. to 200° C. and thereafter reacted with an alkali metal hydroxide solution.

25 12. Aliphatic polyamino amides in which the acid hydrogen attached to the amide nitrogen is replaced by an alkali metal.

30 13. The process of forming aliphatic polyamino amide compounds in which polyamino amides of organic fatty acids of over six carbon atoms are reacted with an alkali metal hydroxide solution at temperatures below 100° C.

35 14. The process of forming a polyamino amide compound in which an organic acid of over six carbon atoms is reacted with diethylene triamine at 130° C. to 200° C. and thereafter reacted with an alkali metal hydroxide solution.

WILLARD L. MORGAN.  
EARLE DAVIS McLEOD.